

# UNITED STATES PATENT OFFICE.

OTTO RÖHM, OF DARMSTADT, GERMANY.

## PROCESS OF DEPILATING AND REDUCING HIDES AND SKINS.

1,082,911.

Specification of Letters Patent. Patented Dec. 30, 1913.

No Drawing.

Application filed December 4, 1911. Serial No. 663,903.

To all whom it may concern:

Be it known that I, OTTO RÖHM, a subject of the Emperor of Germany, residing in Darmstadt, Germany, have invented certain new and useful Improvements in the Process of Depilating and Reducing Hides and Skins, of which the following is a specification.

My invention relates to a method of 10 depilating and reducing, that is, dissolving the so-called scud, of hides and skins by the employment of which the separate processes of liming and bating the hides and skins as now employed in the manufacture of leather 15 are eliminated.

One of the objects, therefore, of my invention, is to decrease the number of processes or steps employed in the manufacture of leather and thereby cause a corresponding 20 decrease in the amount of work necessary to be done.

A further object, which is effected by the elimination of the liming process, is to shorten the time heretofore necessarily required for the two steps or processes of liming and bating employed in the course of the 25 manufacture of leather.

The employment of tryptic enzymes, for instance, the trypsin of the pancreas, in the 30 process of bating hides and skins has heretofore been practised but it was not known prior to my discovery of the fact that the depilation of the hides and skins and the removal of the so-called scud therefrom might 35 and could be effected by treating the same with solutions containing tryptic enzymes, for instance, trypsin of the pancreas. It will be seen, therefore, that by the employment of such solution to take the place of 40 the liming process the latter is completely eliminated, thereby removing one of the heretofore employed steps in the manufacture of leather.

In the practising of my invention the 45 hides or skins which have been soaked in water are placed in a solution of tryptic enzymes, for instance, the trypsin of the pancreas. The action of this solution upon the hides or skins enables the complete removal therefrom of both the hair and the scud.

Although trypsin may be employed alone

in solution I have found that the action thereof is enhanced by employing the same in an alkaline solution.

55

My process may be carried out or practised and the same effect produced by first placing the hides or skins for a short time in an alkaline solution before or after using a solution of trypsin. The action of the 60 trypsin may also be aided by the addition of amino acid.

Putrefaction may, of course, be prevented by the addition of any suitable antiseptic substance.

65

Various advantages result from the treatment of hides or skins with trypsin as above set forth.

As already pointed out, the employment of my invention in the treatment of the 70 hides and skins eliminates entirely the process or step of liming heretofore employed, thereby decreasing not only the amount of work necessary in the operation of manufacturing leather but also decreasing the length of time necessary for the preparation of the hides or skins for the 75 tanning liquor.

Another advantageous result is that the 80 injury to the hair or wool caused by the liming process heretofore employed is obviated so that the by-products of hair and wool are in much better condition and therefore more valuable than they heretofore have been.

85

Furthermore, by the employment of my invention as above set forth the hygienic condition of the beam house is greatly improved to the benefit of the workmen employed therein.

90

Other objects and advantages which will not be mentioned here will suggest themselves to those skilled in the art to which this invention relates.

Having thus described my invention, I 95 claim:

1. The process of depilating and reducing hides and skins which consists in treating the same with a solution of tryptic enzym.
2. The process of depilating and reducing 100 hides and skins which consists in treating the same with an alkaline solution of tryptic enzym.
3. The process of depilating and reducing

hides and skins which consists in soaking the same in water and thereafter treating the same with a solution of tryptic enzym.

4. The process of depilating and reducing 5 hides and skins which consists in soaking the same in water and thereafter treating the same with an alkaline solution of tryptic enzym.

5. The process of depilating and reducing 10 hides and skins which consists in treating them first in an alkaline solution and then with a solution of tryptic enzym.

6. The process of depilating and reducing hides and skins which consists in treating

them with a solution of tryptic enzym and 15 an alkaline solution, the treatment being first with one of the said solutions and being then followed by a treatment with the other solution.

In testimony that I claim the foregoing 20 as my invention, I have hereunto signed my name this 12th day of November, A. D. 1911, at Darmstadt, Germany.

OTTO RÖHM.

In the presence of—

MAX GOLDMANN,  
RICHARD SLAUTTER.